



US006183947B1

**(12) United States Patent**  
**Ito**

**(10) Patent No.:** **US 6,183,947 B1**  
**(45) Date of Patent:** **Feb. 6, 2001**

**(54) PREPARATION METHOD OF ORGANIC SILVER SALT DISPERSION AND THERMALLY PROCESSABLE PHOTOSENSITIVE MATERIAL**

**(75) Inventor:** **Satoshi Ito**, Hino (JP)

**(73) Assignee:** **Konica Corporation** (JP)

**(\*) Notice:** Under 35 U.S.C. 154(b), the term of this patent shall be extended for 0 days.

**(21) Appl. No.:** **09/407,493**

**(22) Filed:** **Sep. 28, 1999**

**(30) Foreign Application Priority Data**

Nov. 9, 1998 (JP) ..... 10-317719

**(51) Int. Cl.<sup>7</sup>** ..... **G03C 1/498**

**(52) U.S. Cl.** ..... **430/619; 430/617; 430/620**

**(58) Field of Search** ..... 430/617, 619, 430/620

**(56) References Cited**

**U.S. PATENT DOCUMENTS**

3,839,049 \* 10/1974 Simons .

\* cited by examiner

*Primary Examiner*—Thorl Chea

*(74) Attorney, Agent, or Firm*—Jordan B. Bierman; Bierman, Muserlian and Lucas

**(57) ABSTRACT**

A method for preparing an organic silver salt dispersion is disclosed, comprising allowing silver nitrate is added to an aqueous solution or suspension of an alkali salt of an organic acid to react to form an organic silver salt dispersion, wherein the aqueous solution or suspension of an alkali salt of an organic acid is cooled at a mean cooling rate of not less than 0.5° C./min. to a temperature of 0° C. to 55° C., and then silver nitrate is added thereto.

**7 Claims, 1 Drawing Sheet**

FIG. 1



FIG. 2



**PREPARATION METHOD OF ORGANIC SILVER SALT DISPERSION AND THERMALLY PROCESSABLE PHOTOSENSITIVE MATERIAL**

**FIELD OF THE INVENTION**

The present invention relates to a method for preparing an organic silver salt dispersion and thermally processable photosensitive materials containing the organic silver salt dispersion prepared by use thereof.

**BACKGROUND OF THE INVENTION**

Methods for preparing an organic silver salt dispersion, which is used as a silver source in thermally processable photosensitive materials, are well known in the art, including a method of preparing organic silver salts in the concurrent presence of water and an organic solvent, as described in JP-A 49-93310, 49-94619 and 53-68702 (herein, the term, JP-A means published unexamined Japanese Patent Application); a method of preparing organic silver salts in an organic solvent, as described in JP-A 57-186745 and 47-9432, and U.S. Pat. No. 3,700,458; and a method of preparing organic silver salts in an aqueous solution, as described in JP-A 53-31611, 54-4117, 54-46709 and U.S. Pat. No. 5,434,043.

There are also known methods for incorporating silver halide into a thermally processable material to provide photosensitivity to the thermally processable material. There have been employed silver halides prepared based on a process of preparing conventional aqueous silver halide gelatin emulsions, which are advantageous in terms of easy introduction of techniques, such as control of the crystal size and crystal habit, impurity doping and chemical ripening. In cases when preparing organic silver salts concurrently in the presence of an organic solvent or in an organic solvent solution, however, it is difficult to allow the silver halide, which has been made water-miscible through gelatin, to be homogeneously dispersed in the organic silver salt dispersion, making it hard to achieve desired photographic characteristics, such as maximum density and sensitivity. Accordingly, in general, silver halide is added at the stage of preparing an organic silver salt in an aqueous solution. Thus, it is advantageous to prepare an organic silver salt dispersion in an aqueous solution.

In the process of preparing an organic silver salt dispersion in an aqueous solution, a fatty acid is dissolved in water at a temperature of higher than its melting point to form a sodium salt, then, after the temperature is lowered, a silver halide emulsion is added and silver nitrate is further added thereto to form an organic silver salt dispersion. Lowering the temperature before adding silver nitrate results in a rapid increase in solution viscosity and addition of silver nitrate also increases the viscosity. In cases when the solution was not uniformly stirred at a high speed, the organic silver salt was non-uniformly formed so that monodispersed fine organic silver salts were not obtained, a thermally processable material prepared by use thereof resulting in problems in performance, such as high fogging levels. It has therefore been desired to solve the problems described above.

**SUMMARY OF THE INVENTION**

Accordingly, an object of the present invention is to provide a method for preparing an organic silver salt dispersion in which organic silver salts are uniformly dispersed, and a thermally processable photosensitive material contain-

ing the organic silver salt dispersion, exhibiting superior photographic performance including enhanced sensitivity and low fogging, and improved image storage stability.

The object of the present invention is achieved by the following constitution:

1. a method for preparing an organic silver salt dispersion comprising the steps of:

- (a) dissolving an organic acid in water at a temperature of 60 to 90° C.,
- (b) adding thereto an alkali to form an aqueous solution or suspension containing an alkali salt of the organic acid,
- (c) cooling the aqueous solution or suspension to a temperature of 0 to 55° C., and then
- (d) adding silver nitrate to the aqueous solution or suspension to form an organic silver salt dispersion, wherein in step (c), the aqueous solution or suspension is cooled at a mean cooling rate of not less than 0.5° C./min; and

2. a thermally processable photosensitive material comprising a support having thereon an organic silver salt, a photosensitive silver halide, a reducing agent and a binder, wherein said organic silver salt is the organic silver salt dispersion prepared by the method described above.

**BRIEF EXPLANATION OF DRAWING**

FIGS. 1 and 2 illustrate sectional view of a reaction used in the preparation method according to the invention.

Explanation of numerals

- 1 Reaction apparatus main body
- 2 Anchor mixer
- 3 Disper mixer
- 4 Disper mixer
- 5 Silver nitrate-introducing pipe
- 6 Homomixer
- 7 Stirring blade
- 8 Fixed ring
- 9 Bearing
- 10 Flowing direction of dispersion
- 11 Jacket
- 12 Motor

**DETAILED DESCRIPTION OF THE INVENTION**

In general, to prepare an aqueous solution or suspension of an alkali salt of an organic acid, the organic acid is dissolved in water at a temperature higher than the melting point of the organic acid (e.g., 60 to 90° C.) and subsequently, an alkali is added thereto to form an alkali salt thereof. Examples of the alkali used in the invention include alkali metal hydroxides and alkali metal carbonates. Specifically, alkali metal hydroxides are preferably used.

In cases when photosensitive silver halide or silver nitrate was further added thereto at a high enough temperature (i.e., 60° C. to 90° C.) to form an organic silver salt dispersion, thermal-fogging tended to occur so that it was necessary to cool the aqueous organic acid alkali salt solution or suspension, which had been maintained at a high temperature, to a temperature of 0° C. to 55° C. In such a case, the viscosity of the aqueous solution or suspension rapidly increased. As a result, it was hard to conduct sufficient stirring in the subsequent preparation of an organic silver salt dispersion with adding silver halide and silver

nitrate, making it difficult to obtain an organic silver salt dispersion at superior dispersing state.

However, it was found that no abrupt rise of viscosity occurs when, prior to addition of silver nitrate, an aqueous solution or suspension of an alkali salt of an organic acid is cooled to a temperature range of 0° C. to 55° C. at a mean cooling rate of not less than 0.5° C./min. Although the details why the application of a specific mean cooling rate prevents an abrupt rise of the viscosity, is not clear, it is presumed that formation of secondary aggregates of the organic acid alkali salt is prevented when cooled at the rate described above.

The mean cooling rate refers to a value of the difference in temperature between before start of cooling and after completion of cooling, divided by the time taken for cooling, as defined below:

$$\text{Mean cooling rate} = (\text{Temperature before cooling} - \text{temperature after cooling}) / \text{Cooling time}$$

The mean cooling rate is preferably 1° C./min. to 100° C./min., more preferably 1.5° C./min. to 50° C./min., and still more preferably 2° C./min. to 10° C./min.

Various methods are applicable as means for cooling in the invention. Examples thereof include a cooling method employing thermal conduction from the side or bottom of a reaction vessel containing an aqueous solution or suspension of an organic acid alkali salt, as well as a cooling method by conventional heat-exchangers such as coil type heat exchanger, double pipe type heat exchanger and multiple pipe type heat exchanger.

The temperature of the aqueous solution or suspension of an organic acid alkali salt at the time of adding silver nitrate is preferably 0° to 55° C., more preferably 10 to 40° C., and still more preferably 20 to 35° C.

In the preparation method of organic silver salt dispersions according to the invention, various stirring means can be used in a reaction apparatus and a high speed stirring machine having a shearing force is preferably employed. Further, to enhance mixing efficiency, a stirrer rotating along the inner wall or bottom of a reaction apparatus may be used in combination with the high speed stirring machine described above.

In FIGS. 1 and 2, anchor mixer 2 is the stirrer rotating along the inner wall or bottom of a reaction apparatus main body 1 and disper mixers 3 and 4 are the high speed stirring machine. In FIG. 2, disper mixer 3 and homo-mixer 6 are each high speed stirring machines.

At least one high speed stirring machine is to be provided in the reaction apparatus used in the invention, and two or more high speed stirring machines be preferably employed.

In cases when two high speed stirring machines are concurrently employed, to obtain an organic silver salt dispersion superior in dispersion uniformity, it is preferred that the high speed stirring members reversely rotate.

Employed as the high speed stirring machine in the invention is preferably a high speed rotating centrifugal radiation type stirring machine (disper mixer 9) or a high speed rotation shearing type stirring machine (homomixer). The high speed rotating centrifugal radiation type stirring machine (also called a disper type stirrer) is a device in which a disc-shaped impeller with circular saw-like edges which are bent alternately up and down, is allowed to rotate enough to cause a vortex to catch up powder into liquid and pulverize powdery aggregates through cutting action of the peripheral edges.

The high speed rotation shearing type stirring machine (also called a homomixer type stirrer) is a device comprised of a combination of a rotatable high speed stirring blade 7

and a fixed ring (stator) provided near the periphery of the stirring blade (as shown in FIG. 2), in which pulverization is carried out employing strong shearing effects or bombarding force produced in the minimal spacing between the stirring blade and the fixed ring.

The circulating speed of the disper mixer or the homomixer is preferably 1 to 100 m/sec, more preferably 1 to 100 m/sec., and still more preferably 1 to 30 m/sec. The circulating speed of the anchor mixer is preferably 0.1 to 10 m/sec, more preferably 0.1 to 5 m/sec., and still more preferably 0.1 to 3 m/sec.

Examples of the reaction apparatus shown in FIGS. 1 and 2 include T.K. Combimix (available from TOKUSHIUKIKAKOOGYO Co. Ltd.), Hybridmixer (available from SATAKE KAGAKUKIKAOKOGYO Co. Ltd.), vacuum emulsifying stirrer (available from MIZUHO KOGYO Co. Ltd.) and vacuum emulsifying disperser FRIMIX (available from SHINKO PANTEX Co. Ltd.).

In the preparation method of organic silver salt dispersions according to the invention, silver nitrate may be added onto the surface or into the interior of the aqueous organic acid alkali salt solution or suspension. To enhance the dispersity of organic silver salts, addition into the interior is preferred and addition into portions near the high speed stirring machine in the reaction mixture solution is more preferred.

Silver nitrate is added preferably within 60 min. (more preferably 30 min., and still more preferably 10 min.) after completion of cooling the aqueous organic acid alkali salt solution or suspension.

Organic silver salts employed in the present invention are reducible silver sources and preferred are organic acids and silver salts of hetero-organic acids having a reducible silver ion source, specifically, long chain (having from 10 to 30 carbon atoms, and preferably from 15 to 25 carbon atoms) aliphatic carboxylic acids and nitrogen-containing heterocyclic ring carboxylic acid. Organic or inorganic silver salt complexes are also useful in which the ligand has a total stability constant for silver ion of 4.0 to 10.0. Examples of preferred silver salts are described in Research Disclosure, Items 17029 and 29963, including organic acid salts (for example, salts of gallic acid, oxalic acid, behenic acid, stearic acid, palmitic acid, lauric acid, etc.); carboxyalkylthiourea salts (for example, 1-(3-carboxypropyl)thiourea, 1-(3-carboxypropyl)-3,3-dimethylthiourea, etc.); silver complexes of polymer reaction products of aldehyde with hydroxy-substituted aromatic carboxylic acid (for example, aldehydes (formaldehyde, acetaldehyde, butylaldehyde, etc.), hydroxy-substituted acids (for example, salicylic acid, benzoic acid, 3,5-dihydroxybenzoic acid, 5,5-thiodisalicylic acid, silver salts or complexes of thiones (for example, 3-(2-carboxyethyl)-4-hydroxymethyl-4-(thiazoline-2-thione and 3-carboxymethyl-4-thiazoline-2-thione), complexes of silver with nitrogen acid selected from imidazole, pyrazole, urazole, 1,2,4-thiazole, and 1H-tetrazole, 3-amino-5-benzylthio-1,2,4-triazole and benztriazole or salts thereof; silver salts of saccharin, 5-chlorosalicylaldoxime, etc.; and silver salts of mercaptides. Of these organic silver salts, silver salts of fatty acids are preferred, and silver salts of behenic acid, arachidinic acid and stearic acid are specifically preferred.

A dispersions of an aqueous organic silver salt used in the invention can be obtained by mixing silver nitrate and an alkali metal salt of an organic acid, and specifically, it is preferred to prepare the dispersion in such a manner that silver halide is added to the alkali metal salt of the organic acid and then silver nitrate is added thereto. For example, to

an organic acid is added an alkali metal hydroxide (e.g., sodium hydroxide, potassium hydroxide, etc.) to form an alkali meat salt soap of the organic acid (e.g., sodium behenate, sodium arachidinate, etc.), thereafter, silver halide is added and then, silver nitrate is further added and subjected to mixing to prepare an aqueous organic silver salt dispersion. Alternatively, the organic acid alkali metal salt, silver nitrate and silver halide may be simultaneously added by the controlled triple jet addition to obtain an aqueous organic silver salt dispersion. Specifically, the preparation of an aqueous organic silver salt dispersion by the controlled triple jet addition is preferred in terms of simplicity of the manufacturing process. Furthermore, the preparation method of an aqueous organic silver salt dispersion by the controlled triple jet addition is preferred also in terms of preparing a thermal processable photosensitive material with enhanced sensitivity.

Silver halide grains of photosensitive silver halide in the present invention work as a light sensor. In order to minimize cloudiness after image formation and to obtain excellent image quality, the less the average grain size, the more preferred, and the average grain size is preferably less than 0.1  $\mu\text{m}$ , more preferably between 0.01 and 0.1  $\mu\text{m}$ , and still more preferably between 0.02 and 0.08  $\mu\text{m}$ . The average grain size as described herein is defined as an average edge length of silver halide grains, in cases where they are so-called regular crystals in the form of cube or octahedron. Furthermore, in cases where grains are not regular crystals, for example, spherical, cylindrical, and tabular grains, the grain size refers to the diameter of a sphere having the same volume as the silver grain.

Furthermore, silver halide grains are preferably monodisperse grains. The monodisperse grains as described herein refer to grains having a monodispersibility obtained by the formula described below of less than 40%; more preferably less than 30%, and most preferably from 0.1 to 20%.

Monodispersibility=(standard deviation of grain diameter)/(average grain diameter)  $\times 100\%$

The silver halide grain shape is not specifically limited, but a high ratio accounted for by a Miller index [100] plane is preferred. This ratio is preferably at least 50%; is more preferably at least 70%, and is most preferably at least 80%. The ratio accounted for by the Miller index [100] face can be obtained based on T. Tani, J. Imaging Sci., 29, 165 (1985) in which adsorption dependency of a [111] face or a [100] face is utilized.

Furthermore, another preferred silver halide shape is a tabular grain. The tabular grain as described herein is a grain having an aspect ratio represented by  $r/h$  of at least 3, wherein  $r$  represents a grain diameter in  $\mu\text{m}$  defined as the square root of the projection area, and  $h$  represents thickness in  $\mu\text{m}$  in the vertical direction. Of these, the aspect ratio is preferably between 3 and 50. The grain diameter is preferably not more than 0.1  $\mu\text{m}$ , and is more preferably between 0.01 and 0.08  $\mu\text{m}$ . These are described in U.S. Pat. Nos. 5,264,337, 5,314,789, 5,320,958, and others. In the present invention, when these tabular grains are used, image sharpness is further improved.

The composition of silver halide may be any of silver chloride, silver chlorobromide, silver chloroiodobromide, silver bromide, silver iodobromide, or silver iodide. The photographic emulsion employed in the present invention can be prepared employing methods described in P. Glafkides, "Chimie et Physique Photographique" (published by Paul Montel Co., 1967), G. F. Duff in, "Photographic Emulsion Chemistry" (published by The Focal Press, 1966), V. L. Zelikman et al., "Making and Coating Photographic Emulsion" (published by The Focal Press, 1964), etc.

Generally, the content of silver halide in organic silver salt is preferably between 0.75 and 30% by weight, based on the organic silver salt.

Silver halide preferably occludes ions of metals belonging to Groups 6 to 11 of the Periodic Table. Preferred as the metals are W, Fe, Co, Ni, Cu, Ru, Rh, Pd, Re, Os, Ir, Pt and Au.

These metals may be introduced into silver halide in the form of a complex. In the present invention, regarding the transition metal complexes, six-coordinate complexes represented by the general formula described below are preferred:

Formula:  $(\text{ML}_6)^m$ :

wherein M represents a transition metal selected from elements in Groups 6 to 11 of the Periodic Table; L represents a coordinating ligand; and m represents 0, 1-, 2-, 3- or 4-. Exemplary examples of the ligand represented by L include halides (fluoride, chloride, bromide, and iodide), cyanide, cyanato, thiocyanato, selenocyanato, tellurocyanato, azido and aquo, nitrosyl, thionitrosyl, etc., of which aquo, nitrosyl and thionitrosyl are preferred. When the aquo ligand is present, one or two ligands are preferably coordinated. L may be the same or different.

The particularly preferred example of M is rhodium (Rh), ruthenium (Ru), rhenium (Re), iridium (Ir) or osmium (Os).

Exemplary examples of transition metal ligand complexes are shown below.

- 1:  $[\text{RhCl}_6]^{3-}$
- 2:  $[\text{RuCl}_6]^{3-}$
- 3:  $[\text{ReCl}_6]^{3-}$
- 4:  $[\text{RuBr}_6]^{3-}$
- 5:  $[\text{OsCl}_6]^{3-}$
- 6:  $[\text{IrCl}_6]^{4-}$
- 7:  $[\text{Ru}(\text{NO})\text{Cl}_5]^{2-}$
- 8:  $[\text{RuBr}_4(\text{H}_2\text{O})]^{2-}$
- 9:  $[\text{Ru}(\text{NO})(\text{H}_2\text{O})\text{Cl}_4]^-$
- 10:  $[\text{RhCl}_5(\text{H}_2\text{O})]^{2-}$
- 11:  $[\text{Re}(\text{NO})\text{Cl}_5]^{2-}$
- 12:  $[\text{Re}(\text{NO})\text{CN}_5]^{2-}$
- 13:  $[\text{Re}(\text{NO})\text{ClC}_4]^{2-}$
- 14:  $[\text{Rh}(\text{NO})_2\text{Cl}_4]^-$
- 15:  $[\text{Rh}(\text{NO})(\text{H}_2\text{O})\text{Cl}_4]^-$
- 16:  $[\text{Ru}(\text{NO})\text{CN}_5]^{2-}$
- 17:  $[\text{Fe}(\text{CN})_6]^{3-}$
- 18:  $[\text{Rh}(\text{NS})\text{Cl}_5]^{2-}$
- 19:  $[\text{Os}(\text{NO})\text{Cl}_5]^{2-}$
- 20:  $[\text{Cr}(\text{NO})\text{Cl}_5]^{2-}$
- 21:  $[\text{Re}(\text{NO})\text{Cl}_5]^-$
- 22:  $[\text{Os}(\text{NS})\text{Cl}_4(\text{TeCN})]^{2-}$
- 23:  $[\text{Ru}(\text{NS})\text{Cl}_5]^{2-}$
- 24:  $[\text{Re}(\text{NS})\text{Cl}_4(\text{SeCN})]^{2-}$
- 25:  $[\text{Os}(\text{NS})\text{Cl}(\text{SCN})_4]^{2-}$
- 26:  $[\text{Ir}(\text{NO})\text{Cl}_5]^{2-}$
- 27:  $[\text{Ir}(\text{NS})\text{Cl}_5]^{2-}$

One type of these metal ions or complex ions may be employed and the same type of metals or the different type of metals may be employed in combinations of two or more types. Generally, the content of these metal ions or complex ions is suitably between  $1 \times 10^{-9}$  and  $1 \times 10^{-2}$  mole per mole of silver halide, and is preferably between  $1 \times 10^{-8}$  and  $1 \times 10^{-4}$  mole.

Compounds, which provide these metal ions or complex ions, are preferably incorporated into silver halide grains through addition during the silver halide grain formation. These may be added during any preparation stage of the silver halide grains, that is, before or after nuclei formation, growth, physical ripening, and chemical ripening. However, these are preferably added at the stage of nuclei formation, growth, and physical ripening; furthermore, are preferably added at the stage of nuclei formation and growth; and are most preferably added at the stage of nuclei formation.

These compounds may be added several times by dividing the added amount. Uniform content in the interior of a silver halide grain can be carried out. As disclosed in JP-A No. 63-29603, 2-306236, 3-167545, 4-76534, 6-110146, 5-273683, the metal can be distributively occluded in the interior of the grain.

These metal compounds can be dissolved in water or a suitable organic solvent (for example, alcohols, ethers, glycols, ketones, esters, amides, etc.) and then added. Furthermore, there are methods in which, for example, an aqueous metal compound powder solution or an aqueous solution in which a metal compound is dissolved along with NaCl and KCl is added to a water-soluble silver salt solution during grain formation or to a water-soluble halide solution; when a silver salt solution and a halide solution are simultaneously added, a metal compound is added as a third solution to form silver halide grains, while simultaneously mixing three solutions; during grain formation, an aqueous solution comprising the necessary amount of a metal compound is placed in a reaction vessel; or during silver halide preparation, dissolution is carried out by the addition of other silver halide grains previously doped with metal ions or complex ions. Specifically, the preferred method is one in which an aqueous metal compound powder solution or an aqueous solution in which a metal compound is dissolved along with NaCl and KCl is added to a water-soluble halide solution. When the addition is carried out onto grain surfaces, an aqueous solution comprising the necessary amount of a metal compound can be placed in a reaction vessel immediately after grain formation, or during physical ripening or at the completion thereof or during chemical ripening.

Silver halide grain emulsions used in the invention may be desalinated after the grain formation, using the methods known in the art, such as the noodle washing method and flocculation process.

The photosensitive silver halide grains used in the invention is preferably subjected to a chemical sensitization. As preferable chemical sensitizations, well known chemical sensitizations in this art such as a sulfur sensitization, a selenium sensitization and a tellurium sensitization are usable. Furthermore, a noble metal sensitization using gold, platinum, palladium and iridium compounds and a reduction sensitization are available. As the compounds preferably used in the sulfur sensitization, the selenium sensitization and the tellurium sensitization, well known compounds can be used and the compounds described in JP-A No. 7-128768 is usable. Examples of useful tellurium sensitizers include diacyltellurides, bis(oxycarbonyl)tellurides, bis(carbamoyl) tellurides, bis(oxycarbonyl)ditellurides, bis(carbamoyl) ditellurides, compounds containing P=Te bond, tellurocarboxylic acids, Te-organictellurocarboxylic acid esters, di(poly)tellurides, tellurides, tellurols, telluroacetals, tellurosulfonates, compounds containing P-Te bond, Te containing heterocyclic ring compounds, tellurocarbonyl compounds, inorganic tellurium compounds and colloidal tellurium, etc. Examples of the compounds used in the noble

metal sensitization include chloroauric acid, potassium chloroaurate, potassium aurothiocyanate, gold sulfide, gold selenide, compounds described U.S. Pat. No. 2,448,060 and British Patent No. 618,061.

Examples of the compounds used in the reduction sensitization include ascorbic acid, thiourea dioxide, stannous chloride, aminoiminomethanesulfonic acid, hydrazine derivatives, borane compounds, silane compounds and polyamine compounds. The reduction sensitization can be carried out by ripening an emulsion of which pH and pAg are kept to not less than 7 and not more than 8.3 respectively. Furthermore, the reduction sensitization can be carried out by introducing a single addition part of silver ion during the grains being formed.

Reducing agents are preferably incorporated into the thermally processable photosensitive material of the present invention. Examples of suitable reducing agents are described in U.S. Pat. Nos. 3,770,448, 3,773,512, and 3,593,863, and Research Disclosure Items 17029 and 29963, and include the following: aminohydroxycycloalkenone compounds (for example, 2-hydroxypiperidino-2-cyclohexane); esters of amino reductones as the precursor of reducing agents (for example, piperidinohexose reducton monoacetate); N-hydroxyurea derivatives (for example, N-p-methylphenyl-N-hydroxyurea); hydrazones of aldehydes or ketones (for example, anthracenealdehyde phenylhydrazone; phosphamidophenols; phosphamidoanilines; polyhydroxybenzenes (for example, hydroquinone, t-butylhydroquinone, isopropylhydroquinone, and (2,5-dihydroxy-phenyl)methylsulfone); sulphydroxamic acids (for example, benzenesulphydroxamic acid); sulfonamidoanilines (for example, 4-(N-methanesulfonamide)aniline); 2-tetrazolylthiohydroquinones (for example, 2-methyl-5-(1-phenyl-5-tetrazolylthio)hydroquinone); tetrahydroquinon-oxalines (for example, 1,2,3,4-tetrahydroquinoxaline); amidoxines; azines (for example, combinations of aliphatic carboxylic acid arylhydrazides with ascorbic acid); combinations of polyhydroxybenzenes and hydroxylamines, reductones and/or hydrazine; hydroxamic acids; combinations of azines with sulfonamidoanilines;  $\alpha$ -cyanophenylacetic acid derivatives; combinations of bis- $\beta$ -naphthol with 1,3-dihydroxybenzene derivatives; 5-pyrazolones, sulfonamidophenol reducing agents, 2-phenylindane-1,3-dione, etc.; chroman; 1,4-dihydropyridines (for example, 2,6-dimethoxy-3,5-dicarboethoxy-1,4-dihydropyridine); bisphenols (for example, bis(2-hydroxy-3-t-butyl-5-methylphenyl)methane, bis(6-hydroxy-m-tri)mesitol, 2,2-bis(4-hydroxy-3-methylphenyl)propane, 4,5-ethylidene-bis(2-t-butyl-6-methyl)phenol, UV-sensitive ascorbic acid derivatives and 3-pyrazolidones. Of these, particularly preferred reducing agents are hindered phenols. As hindered phenols, listed are compounds represented by the general formula (A) described below:



Formula (A)

65 wherein R represents a hydrogen atom or an alkyl group having from 1 to 10 carbon atoms (for example,  $-\text{C}_4\text{H}_9$ , 2,4,4-trimethylpentyl), and R' and R'' each represents an

alkyl group having from 1 to 5 carbon atoms (for example, methyl, ethyl, t-butyl).

Exemplary examples of the compounds represented by 5 the formula (A) are shown below.



A-1

10



A-2



A-3



A-4



A-5



A-6

-continued

A-7



10

The used amount of reducing agents represented by the above-mentioned general formula (A) is preferably between  $1 \times 10^{-2}$  and 10 moles, and is more preferably between 15  $1 \times 10^{-2}$  and 1.5 moles per mole of silver.

Antifoggants may be incorporated into the thermally processable photosensitive material to which the present invention is applied. The substance which is known as the most effective antifoggant is a mercury ion. The incorporation of mercury compounds as the antifoggant into photosensitive materials is disclosed, for example, in U.S. Pat. No. 3,589,903. However, mercury compounds are not environmentally preferred. As mercury-free antifoggants, preferred are those antifoggants as disclosed in U.S. Pat. Nos. 4,546,075 and 4,452,885, and Japanese Patent Publication Open to 25 Public Inspection No. 59-57234.

Particularly preferred mercury-free antifoggants are heterocyclic compounds having at least one substituent, represented by  $-\text{C}(\text{X}1)(\text{X}2)(\text{X}3)$  (wherein X1 and X2 each represent halogen, and X3 represents hydrogen or halogen), 30 as disclosed in U.S. Pat. Nos. 3,874,946 and 4,756,999. As examples of suitable antifoggants, employed preferably are compounds described in paragraph numbers [0030] through [0036] of JP-A No. 9-288328. Further, as another examples of suitable antifoggants, employed preferably are compounds described in paragraph numbers [0062] and [0063] 35 of JP-A No. 9-90550. Furthermore, other suitable antifoggants are disclosed in U.S. Pat. No. 5,028,523, and U.K. Patent Application Nos. 92221383. No. 4, 9300147. No. 7, and 9311790. No. 1.

40 Image toning agents are preferably incorporated into the thermally processable photosensitive material used in the present invention. Examples of preferred image toning agents are disclosed in Research Disclosure Item 17029, and include the following:

45 imides (for example, phthalimide), cyclic imides, pyrazoline-5-one, and quinazolinone (for example, succinimide, 3-phenyl-2-pyrazoline-5-on, 1-phenylurazole, quinazoline and 2,4-thiazolidione); naphthalimides (for example, N-hydroxy-1,8-naphthalimide); cobalt complexes 50 (for example, cobalt hexaminetrifluoroacetate), mercaptans (for example, 3-mercaptop-1,2,4-triazole); N-(aminomethyl) arylidicarboxyimides (for example, N-(dimethylaminomethyl)phthalimide); blocked pyrazoles, 55 isothiuronium derivatives and combinations of certain types of light-bleaching agents (for example, combination of N,N'-hexamethylene(1-carbamoyl-3,5-dimethylpyrazole), 1,8-(3,6-dioxaoctane)bis-(isothiuroniumtrifluoroacetate), and 2-(tribromomethylsulfonyl)benzothiazole; merocyanine dyes (for example, 3-ethyl-5-((3-ethyl-2- 60 benzothiazolinylidene(benzothiazolinylidene))-1-methylethylidene-2-thio-2,4-oxazolidinedione); phthalazinone, phthalazinone derivatives or metal salts thereof (for example, 4-(1-naphthyl)phthalazinone, 6-chlorophthalazinone, 5,7-dimethylphthalazinone, and 2,3-

65

dihydro-1,4-phthalazinedione); combinations of phthalazine and sulfinic acid derivatives (for example, 6-chlorophthalazinone and benzenesulfinic acid sodium, or 8-methylphthalazinone and p-trisulfonic acid sodium); combinations of phthalazine and phthalic acid; combinations of phthalazine (including phthalazine addition products) with at least one compound selected from maleic acid anhydride, and phthalic acid, 2,3-naphthalenedicarboxylic acid or o-phenylenic acid derivatives and anhydrides thereof (for example, phthalic acid, 4-methylphthalic acid, 4-nitrophthalic acid, and tetrachlorophthalic acid anhydride); quinazolinediones, benzoxazine, naphthoxazine derivatives, benzoxazine-2,4-diones (for example, 1,3-benzoxazine-2,4-dione); pyrimidines and asymmetry-triazines (for example, 2,4-dihydroxypyrimidine), and tetraazapentalene derivatives (for example, 3,6-dimercapto-1,4-diphenyl-1H,4H-2,3a,5,6a-tetraazapentalene). Preferred image color control agents include phthalazone or phthalazine.

In the thermally processable photosensitive material of the present invention, employed can be sensitizing dyes described, for example, in JP-A Nos. 63-159841, 60-140335, 63-231437, 63-259651, 63-304242, and 63-15245; U.S. Pat. Nos. 4,639,414, 4,740,455, 4,741,966, 4,751,175, and 4,835,096. Useful sensitizing dyes employed in the present invention are described, for example, in publications described in or cited in Research Disclosure Items 17643, Section IV-A (page 23, December 1978). Particularly, selected can advantageously be sensitizing dyes having the spectral sensitivity suitable for spectral characteristics of light sources of various types of scanners. For example, compounds described in JP-A Nos. 9-34078, 9-54409 and 9-80679 are preferably employed.

In the present invention, to restrain or accelerate development for the purpose of controlling the development, to enhance the spectral sensitive efficiency, or to enhance the reservation stability before and after the development, a mercapto compound, a disulfide compound and a thione compound can be incorporated in the photosensitive material. In cases where the mercapto compound is used in the present invention, any compound having a mercapto group can be used, but preferred compounds are represented by the following formulas, Ar—SM and Ar—S—S—Ar, wherein M represents a hydrogen atom or an alkaline metal atom, Ar represents an aromatic ring compound or a condensed aromatic ring compound having at least a nitrogen, sulfur, oxygen, selenium or tellurium. Preferable aromatic heterocyclic ring compounds include benzimidazole, naphthimidazole, benzothiazole, naphthothiazole, benzoxazole, naphthoxazole, benzoselenazole, benzotellurazole, imidazole, oxazole, pyrazole, triazole, thiadiazole, tetrazole, triazine, pyrimidine, pyridazine, pyrazine, pyridine, purine, quinoline or quinazoline. These aromatic heterocyclic ring compounds may contain a substituent selected from a halogen atom (e.g., Br and Cl), a hydroxy group, an amino group, a carboxy group, an alkyl group (e.g., alkyl group having at least a carbon atom, preferably 1 to 4 carbon atoms) and an alkoxy group (e.g., alkoxy group having at least a carbon atom, preferably 1 to 4 carbon atoms). Examples of mercapto-substituted aromatic heterocyclic ring compounds include 2-mercaptopbenzimidazole, 2-mercaptopbenzoxazole, 2-mercaptopbenzothiazole, 2-mercaptop-5-methylbenzothiazole, 3-mercaptop-1,2,4-triazole, 2-mercaptopquinoline, 8-mercaptopurine, 2,3,5,6-tetrachloro-4-pyridinethiol, 4-hydroxy-2-mercaptopurine, and 2-mercaptop-4-phenyloxazole, but

the exemplified compounds according to the present invention are not limited thereto.

In the present invention, a matting agent is preferably incorporated into the photosensitive layer side. In order to minimize the image abrasion after thermal development, the matting agent is provided on the surface of a photosensitive material and the matting agent is preferably incorporated in an amount of 0.5 to 10 per cent in weight ratio with respect to the total binder in the emulsion layer side.

Materials of the matting agents employed in the present invention may be either organic substances or inorganic substances. Regarding inorganic substances, for example, those can be employed as matting agents, which are silica described in Swiss Patent No. 330,158, etc.; glass powder described in French Patent No. 1,296,995, etc.; and carbonates of alkali earth metals or cadmium, zinc, etc. described in U.K. Patent No. 1,173,181, etc. Regarding organic substances, as organic matting agents those can be employed which are starch described in U.S. Pat. No. 2,322,037, etc.; starch derivatives described in Belgian Patent No. 625,451, U.K. Patent No. 981,198, etc.; polyvinyl alcohols described in Japanese Patent Publication No. 44-3643, etc.; polystyrenes or polymethacrylates described in Swiss Patent No. 330,158, etc.; polyacrylonitriles described in U.S. Pat. No. 3,079,257, etc.; and polycarbonates described in U.S. Pat. No. 3,022,169.

The shape of the matting agent may be crystalline or amorphous. However, a crystalline and spherical shape is preferably employed. The size of a matting agent is expressed in the diameter of a sphere which has the same volume as the matting agent. The particle diameter of the matting agent in the present invention is referred to the diameter of a spherical converted volume. The matting agent employed in the present invention preferably has an average particle diameter of 0.5 to 10  $\mu\text{m}$ , and more preferably of 1.0 to 8.0  $\mu\text{m}$ . Furthermore, the variation coefficient of the size distribution is preferably not more than 50 percent, is more preferably not more than 40 percent, and is most preferably not more than 30 percent. The variation coefficient of the size distribution as described herein is a value represented by the formula described below:

$$\text{Standard deviation of particle diameter}/(\text{average particle diameter}) \times 100$$

The matting agent according to the present invention can be incorporated into arbitrary construction layers. In order to accomplish the object of the present invention, the matting agent is preferably incorporated into construction layers other than the photosensitive layer, and is more preferably incorporated into the farthest layer from the support surface.

Addition methods of the matting agent according to the present include those in which a matting agent is previously dispersed into a coating composition and is then coated, and prior to the completion of drying, a matting agent is sprayed. When a plurality of matting agents are added, both methods may be employed in combination.

In the present invention, to improve an electrification property, a conducting compound such as a metal oxide and/or a conducting polymer can be incorporated into a construction layer. These compounds can be incorporated into any layer, preferably into a sublayer, a backing layer and an intermediate layer between a photosensitive layer and a sublayer, etc. In the present invention, the conducting compounds described in U.S. Pat. No. 5,244,773, column 14 through 20, are preferably used.

Various kinds of additives can be incorporated into a photosensitive layer, a non-photosensitive layer or other construction layers. Except for the compounds mentioned

above, surface active agents, antioxidants, stabilizers, plasticizers, UV (ultra violet rays) absorbers, covering aids, etc. may be employed in the thermally developable photosensitive material according to the present invention. These additives along with the above-mentioned additives are described in Research Disclosure Item 17029 (on page 9 to 15, June, 1978) and can be employed.

Binders suitable for the thermally processable photosensitive material to which the present invention is applied are transparent or translucent, and generally colorless. Binders are natural polymers, synthetic resins, and polymers and copolymers, other film forming media; for example, gelatin, gum arabic, poly(vinyl alcohol), hydroxyethyl cellulose, cellulose acetate, cellulose acetatebutyrate, poly (vinylpyrrolidone), casein, starch, poly(acrylic acid), poly (methylmethacrylic acid), poly(vinyl chloride), poly (methacrylic acid), copoly(styrene-maleic acid anhydride), copoly(styrene-acrylonitrile, copoly(styrene-butadiene, poly (vinyl acetal) series (for example, poly(vinyl formal) and poly(vinyl butyral), poly(ester) series, poly(urethane) series, phenoxy resins, poly(vinylidene chloride), poly(epoxide) series, poly(carbonate) series, poly(vinyl acetate) series, cellulose esters, poly(amide) series. These may be hydrophilic or hydrophobic. In the present invention, the amount of the binder in a photosensitive layer is preferably between 1.5 and 6 g/m<sup>2</sup>, and is more preferably between 1.7 and 5 g/m<sup>2</sup>.

Supports employed in the present invention are preferably, in order to minimize the deformation of images after development processing, plastic films (for example, polyethylene terephthalate, polycarbonate, polyimide, nylon, cellulose triacetate, polyethylene naphthalate).

Of these, as preferred supports, listed are polyethylene terephthalate (hereinafter referred to as PET) and other plastics (hereinafter referred to as SPS) comprising styrene series polymers having a syndiotactic structure. The thickness of the support is between about 50 and about 300  $\mu\text{m}$ , and is preferably between 70 and 180  $\mu\text{m}$ . Furthermore, thermally processed plastic supports may be employed. As acceptable plastics, those described above are listed. The thermal processing of the support, as described herein, is that after film casting and prior to the photosensitive layer coating, these supports are heated to a temperature at least 30° C. higher than the glass transition point, preferably by not less than 35° C. and more preferably by at least 40° C. However, when the supports are heated at a temperature higher than the melting point, no advantages of the present invention are obtained.

Plastics employed in the present invention are described below. PET is a plastic in which all the polyester components are composed of polyethylene terephthalate. However, other than polyethylene terephthalate, employed also may be polyesters in which modified polyester components such as acid components, terephthalic acid, naphthalene-2,6-dicarboxylic acid, isophthalic acid, butylenecarboxylic acid, 5-sodiumsulfoisophthalic acid, adipic acid, etc., and as glycol components, ethylene glycol, propylene glycol, butanediol, cyclohexane dimethanol, etc. may be contained in an amount of no more than 10 mole percent, with respect to the total polyester content. SPS is different from normal polystyrene (atactic polystyrene) and a polystyrene having stereoregularity. The stereoregular structure portion of SPS is termed a racemo chain and the more regular parts increase as 2 chains, 3 chains, 5 chains or more chains, the higher being, the more preferred. In the present invention, the racemo chains are preferably not less than 85 percent for two chains, not less than 75 percent for three chains, not less than

50 percent for five chains, and 30 percent for not less than 5 chains. SPS can be polymerized in accordance with a method described in Japanese Patent Publication Open to Public Inspection No. 3-131843.

As the base casting method of the support and subbing production method which are associated with the present invention, any of those known in the art can be employed. However, those methods described in paragraphs [0030] through [0070] of Japanese Patent Publication Open to Public Inspection No. 9-50094 are preferably employed.

The thermally developable photosensitive material according to the invention, to which the present invention is applied, is subjected to formation of photographic images employing thermal development processing and preferably comprises a reducible silver source (organic silver salt), a photosensitive silver halide with an catalytically active amount, a hydrazine derivative, a reducing agent and, if desired, an image color control agent, to adjust silver tone, which are generally dispersed into a (organic) binder matrix.

The thermally developable photosensitive material according to the invention is stable at normal temperatures and is developed, after exposure, when heated (for example, to 80 to 140° C.). Upon heating, silver is formed through an oxidation-reduction reaction between the organic silver salt

(functioning as an oxidizing agent) and the reducing agent. This oxidation-reduction reaction is accelerated by the catalytic action of a latent image formed in the silver halide through exposure. Silver formed by the reaction with the organic silver salt in an exposed area yields a black image, which contrasts with an unexposed area to form an image. This reaction process proceeds without the further supply of a processing solution such as water, etc. from outside.

The thermally developable photosensitive material according to the invention comprises a support having thereon at least one photosensitive layer, and the photosensitive layer may only be formed on the support. Further, at least one non-photosensitive layer is preferably formed on the photosensitive layer. In order to control the amount or wavelength distribution of light transmitted through the photosensitive layer, a filter layer may be provided on the same side as the photosensitive layer, and/or an antihalation layer, that is, a backing layer on the opposite side. Dyes or pigments may also be incorporated into the photosensitive layer. As the usable dyes, those which can absorb aimed wavelength in desired wavelength region can be used, preferred are compounds described in JP-A Nos. 59-6481, 59-182436, U.S. Pat. No. 4,594,312, European Patent Publication Nos. 533,008, 652,473, JP-A Nos. 2-216140, 4-348339, 7-191432, 7-301890.

Furthermore, these non-photosensitive layers may contain the above-mentioned binder, a matting agent and a lubricant such as a polysiloxane compound, a wax and a liquid paraffin.

The photosensitive layer may be composed of a plurality of layers. Furthermore, for gradation adjustment, in terms of sensitivity, layers may be constituted in such a manner as a fast layer/slow layer or a slow layer/fast layer.

Details of the thermally developable photosensitive materials are disclosed, as described above, in, for example, in U.S. Pat. Nos. 3,152,904 and 3,457,075, and D. Morgan, "Dry Silver Photographic Material" and D. Morgan and B. Shely, "Thermally Processed Silver Systems" (Imaging Processes and Materials) Neblette, 8th Edition, edited by Sturge, V. Walworth, and A. Shepp, page 2, 1969), etc. Of these, the thermally developable photosensitive material used in the invention is characterized in that they are thermally developed at temperature of 80 to 140° C. so as to

15

obtain images without fixation, so that the silver halide and the organic silver salt in an unexposed portion are not removed and remain in the photosensitive materials.

In the present invention, it is preferred that optical transmission density of the photosensitive material including a support at 400 nm after thermally developed is preferably not more than 0.2, more preferably 0.02 to 0.2. With the optical transmission density of less than 0.02, sensitivity is too low to meet a practical use.

#### EXAMPLES

The present invention will be further explained based on examples, but embodiments of the present invention are not limited to these examples.

##### Example 1

###### Preparation of silver halide emulsion A

In 900 ml of deionized water were dissolved 7.5 g of gelatin and 10 mg of potassium bromide. After adjusting the temperature and the pH to 35° C. and 3.0, respectively, 370 ml of an aqueous solution containing 74 g silver nitrate and  $1 \times 10^{-4}$  mol/mol Ag of  $K_2Ir(NO)_5Cl_5$  and an equimolar aqueous solution containing potassium bromide and potassium iodide in a molar ratio of 98 to 2 were added over a period of 10 minutes by the controlled double-jet method, while the pAg was maintained at 7.7. Thereafter, 4-hydroxy-6-methyl-1,3,3a,7-tetraazaindene was added and the pH was adjusted to 5 using NaOH. There was obtained cubic silver iodobromide grains having an average grain size of 0.06  $\mu$ m, a variation coefficient of the projection area equivalent diameter of 11 percent, and the proportion of the {100} face of 87 percent. The resulting emulsion was flocculated to remove soluble salts, employing a flocculating agent and after desalting, 0.1 g of phenoxyethanol was added and the pH and pAg were adjusted to 5.9 and 7.5, respectively. Then, sodium thiosulfate and chloroauric acid were added and ripening was carried out to obtain silver halide emulsion A.

###### Preparation of fatty acid sodium salt B1

Using Combimix type SL-10, produced by TOKUSHI-UKIKAKO GYO Co. Ltd. (as illustrated in FIG. 1), the following procedure was conducted. In the reaction vessel of the Combimix type SL-10, 212.0 g of behenic acid, 29.2 g of arachidinic acid and 8.85 g of stearic acid were dissolved in 4750 ml of water at 90° C., while anchor mixer 2 was operated at a rotation speed of 100 rpm, and disper mixers 3 and 4 each were operated at 1,500 rpm in the same direction. Subsequently, 748.5 ml of an aqueous 1.0M sodium hydroxide solution was added thereto. After adding 6.9 ml of concentrated nitric acid, the reaction mixture was cooled to 30° C. over a period of 10 min. (i.e., mean cooling rate of 6.0° C./min.) by flowing cooling water into jacket 11 of the main body 1 of the reaction apparatus to obtain a fatty acid sodium salt solution B1.

###### Preparation of fatty acid sodium salt B2

Aqueous fatty acid sodium salt solution B2 was prepared in the same manner as B1, except that the reaction mixture was cooled to 30° C. over 30 min.

###### Preparation of fatty acid sodium salt B3

Aqueous fatty acid sodium salt solution B3 was prepared in the same manner as B1, except that the reaction mixture was cooled to 30° C. over 60 min.

###### Preparation of fatty acid sodium salt B4

Aqueous fatty acid sodium salt solution B4 was prepared in the same manner as B1, except that the reaction mixture was cooled to 30° C. over 120 min.

###### Preparation of fatty acid sodium salt B5

Aqueous fatty acid sodium salt solution B5 was prepared in the same manner as B1, except that the reaction mixture was cooled to 30° C. over 150 min.

16

###### Preparation of fatty acid sodium salt B6

Aqueous fatty acid sodium salt solution B6 was prepared in the same manner as B1, except that the reaction mixture was cooled to 55° C. over 90 min.

###### Preparation of organic silver salt dispersion C1

Silver halide emulsion A of 38.1 g and 450 ml of water were added to aqueous fatty acid sodium salt solution B1 maintained at 30° C., while anchor mixer 2 was operated at a rotation speed of 120 rpm and disper mixers 3 and 4 was operated at 2,500 rpm. Then, after setting the rotation speed of anchor mixer 2 at 0 rpm and disper mixers 3 and 4 at 5,000 rpm, 747 ml of 1M silver nitrate solution was added, over a period of 2 min., to the vicinity of the disper mixer 3, provided that the silver nitrate solution was added at 10 min. or earlier after completion of cooling the fatty acid sodium salt solution. After varying again the rotation speed of the disper mixers 3 and 4 to 4,500 rpm, stirring further continued for 10 min. to obtain an organic silver salt dispersion. Thereafter, the resulting organic silver salt dispersion was transferred to a vessel with a volume of 30 lit., water was added with stirring, the mixture was allowed to stand and the silver salt dispersion was separated by floatation. After floatation separation, the lower water layer was removed to remove aqueous soluble salts. Then, water was further removed by a centrifugal dehydrator and the residue was dried at 40° C. over a period of 72 hrs. to obtain a powdery organic silver salt dispersion.

###### Preparation of organic silver salt dispersion C2

Organic silver salt dispersion C2 was prepared in the same manner as C1, except that fatty acid sodium salt solution B1 was replaced by B2.

###### Preparation of organic silver salt dispersion C3

Organic silver salt dispersion C3 was prepared in the same manner as C1, except that fatty acid sodium salt solution B1 was replaced by B3.

###### Preparation of organic silver salt dispersion C4

Organic silver salt dispersion C4 was prepared in the same manner as C1, except that fatty acid sodium salt solution B1 was replaced by B4.

###### Preparation of organic silver salt dispersion C5

Preparation of organic silver salt dispersion C5 was attempted in the same manner as C1, except that fatty acid sodium salt solution B1 was replaced by B5. However, the viscosity of the reaction mixture solution was abruptly raised to be solidified. As a result, silver salt dispersion B5 was not obtained.

###### Preparation of organic silver salt dispersion C6

Organic silver salt dispersion C6 was prepared in the same manner as C1, except that fatty acid sodium salt solution B1 was replaced by B6.

###### Evaluation of organic silver salt dispersion

###### Measurement of grain size

Each of dried powdery organic silver salt dispersions was observed by a transmission electronmicroscope and the grain size of 1,000 grains were measured at random to determine the mean major axis diameter and the mean minor axis diameter.

###### Measurement of dispersity

Homogeneity of the grain diameter (i.e., major axis diameter) distribution of each dispersion was determined, based on the following formula:

$$\text{Monodispersity} = (\text{Standard deviation of grain diameter}) / (\text{mean grain diameter}) \times 100$$

The mean major axis diameter, the mean minor axis diameter and the monodispersity of each organic silver salt

dispersion were shown in Table 1. In addition, the viscosity of the fatty acid sodium salt solution was also shown. Using type B viscometer (available from TOKYOKEIKI Co. Ltd.) and Nos. 1 to 4 rotor at 6 to 60 rpm and a temperature of 30° C., the viscosity was measured within 30 min. after completion of cooling each of fatty acid sodium salt solutions, provided that solution C6 was measured at 55° C.

-continued

5 Butyl acrylate (30 weight %)  
t-butyl acrylate (20 weight %)  
2-Hydroxyethyl acrylate  
(25 weight %)

TABLE 1

| Silver salt dispersion | Viscosity of fatty acid sodium salt solution (cp) | Mean major axis diameter (μm) | Mean minor axis diameter (μm) | Monodispersity (%) | Mean cooling rate (° C./min.) | Remark |
|------------------------|---------------------------------------------------|-------------------------------|-------------------------------|--------------------|-------------------------------|--------|
| C1                     | 2.00                                              | 0.68                          | 0.03                          | 11.00              | 6                             | Inv.   |
| C2                     | 5.00                                              | 0.70                          | 0.03                          | 12.00              | 2                             | Inv.   |
| C3                     | 10.00                                             | 0.80                          | 0.04                          | 14.00              | 1                             | Inv.   |
| C4                     | 100.00                                            | 1.10                          | 0.05                          | 16.00              | 0.5                           | Inv.   |
| C5                     | Non-measurable                                    | —                             | —                             | —                  | 0.4                           | Comp.  |
| C6                     | 1000.0                                            | 1.80                          | 0.15                          | 38.00              | 0.39                          | Comp.  |

As apparent from Table 1, organic silver salt dispersions prepared according to the present invention exhibited a smaller mean diameter and enhanced monodispersity.

25 Example 2  
Preparation of photosensitive emulsion E1

Dried organic silver salt dispersion C1 of 125 g, 3.6 g of polyvinyl butyral (average molecular weight of 4,000) and 363 g of methyl ethyl ketone were mixed with stirring and dispersed at 4,000 psi to obtain photosensitive emulsion E1.

Preparation of photosensitive emulsion E2

Photosensitive emulsion E2 was prepared in the same manner as E1, except that organic silver salt dispersion C1 was replaced by C2.

Preparation of photosensitive emulsion E3

Photosensitive emulsion E3 was prepared in the same manner as E1, except that organic silver salt dispersion C1 was replaced by C3.

Preparation of photosensitive emulsion E4

Photosensitive emulsion E4 was prepared in the same manner as E1, except that organic silver salt dispersion C1 was replaced by C4.

Preparation of photosensitive emulsion E6

Photosensitive emulsion E6 was prepared in the same manner as E1, except that organic silver salt dispersion C1 was replaced by C6.

Preparation of a Subbed PET Photographic Support

Both surfaces of a biaxially stretched thermally fixed 100 μm PET film, available on the market, was subjected to corona discharging at 8 w/m<sup>2</sup>·min. Onto the surface of one side, the subbing coating composition a-1 described below was applied so as to form a dried layer thickness of 0.8 μm, which was then dried. The resulting coating was designated Subbing Layer A-1. Onto the opposite surface, the subbing coating composition b-1 described below was applied to form a dried layer thickness of 0.8 μm. The resulting coating was designated Subbing Layer B-1.

-continued

(C-1)  
Hexamethylene-1,6-bis (ethylenurea)  
Water to make  
Subbing Coating Composition b-1

0.6 g  
0.8 g  
1 liter

Latex liquid (solid portion of 30%)  
of a copolymer consisting of  
butyl acrylate (40 weight %)  
styrene (20 weight %)  
glycidyl acrylate  
(25 weight %)  
(C-1)  
Hexamethylene-1,6-bis (ethylenurea)  
Water to make

270 g  
0.6 g  
0.8 g  
1 liter

Subsequently, the surfaces of Subbing Layers A-1 and B-1 40 were subjected to corona discharging with 8 w/m<sup>2</sup>·minute. Onto the Subbing Layer A-1, the upper subbing layer coating composition a-2 described below was applied so as to form a dried layer thickness of 0.8 μm, which was designated Subbing Layer A-2, while onto the Subbing Layer B-1, the upper subbing layer coating composition b-2 45 was applied so as to form a dried layer thickness of 0.8 μm, having a static preventing function, which was designated Subbing Upper Layer B-2.

|    |                                                              |                                                                |
|----|--------------------------------------------------------------|----------------------------------------------------------------|
| 50 | Upper Subbing Layer Coating Composition a-2                  |                                                                |
| 55 | Gelatin<br>(C-1)<br>(C-2)<br>(C-3)                           | amount to make 0.4 g/m <sup>2</sup><br>0.2 g<br>0.2 g<br>0.1 g |
| 60 | Silica particles (average diameter of 3 μm)<br>Water to make | 0.1 g<br>1 liter                                               |
| 65 | Upper Subbing Layer Coating Composition b-2                  |                                                                |

(C-4)  
Latex solution (solid portion of 20%)  
comprising (C-5) as a substituent  
Ammonium sulfate  
(C-6)  
Polyethylene glycol (average molecular

60 g  
80 g  
0.5 g  
12 g  
6 g

Subbing Coating Composition a-1

Latex solution (with a solid portion of 30%)  
of a copolymer consisting of



-continued



## Emulsion side coating

## Photosensitive layer 1

The following composition was coated so as to have silver coverage of 2.1 g/m<sup>2</sup>.

---

|                                                             |         |
|-------------------------------------------------------------|---------|
| Photosensitive emulsion, as shown in Table 2                | 240 g   |
| Sensitizing dye-1 (0.1% methanol solution)                  | 1.7 ml  |
| Pyridinium bromide perbromide<br>(6% methanol solution)     | 3 ml    |
| Calcium bromide (0.1% methanol solution)                    | 1.7 ml  |
| Antifoggant-2 (10% methanol solution)                       | 1.2 ml  |
| 2-(4-Chlorobenzoyl)-benzoic acid<br>(12% methanol solution) | 9.2 ml  |
| 2-Mercaptobenzimidazole<br>(1% methanol solution)           | 11 ml   |
| Tribromomethylsulfoquinoline<br>(5% methanol solution)      | 17 ml   |
| Reducing agent A-4<br>(20% methanol solution)               | 29.5 ml |
| Contrast-increasing agent H<br>(1% methanol solution)       | 3 ml    |
| Sensitizing dye-1                                           |         |

---



Antifoggant-2

-continued



Contrast-increasing agent H



## Surface protective layer

The following composition was coated on the photosensitive layer.

|                                                                                                |                       |
|------------------------------------------------------------------------------------------------|-----------------------|
| Acetone                                                                                        | 35 ml/m <sup>2</sup>  |
| Methyl ethyl ketone                                                                            | 17 ml/m <sup>2</sup>  |
| Cellulose acetate                                                                              | 2.3 g/m <sup>2</sup>  |
| Methanol                                                                                       | 7 ml/m <sup>2</sup>   |
| Phthalazinone                                                                                  | 250 mg/m <sup>2</sup> |
| 4-Methylphthalic acid                                                                          | 180 mg/m <sup>2</sup> |
| Tetrachlorophthalic acid                                                                       | 150 mg/m <sup>2</sup> |
| Tetrachlorophthalic acid anhydride                                                             | 170 mg/m <sup>2</sup> |
| Matting agent, monodispersed silica having mono-dispersity of 10% and a mean size of 4 $\mu$ m | 70 mg/m <sup>2</sup>  |
| $C_9H_{19}-C^6H^4-SO_3Na$                                                                      | 10 mg/m <sup>2</sup>  |

## Evaluation of photosensitive material

## Exposure and Processing

Thermally processable photosensitive material samples were exposed using an imager having a semiconductor laser of 810 nm and then heat-developed at 120° C. over a period of 15 sec., using an automatic processor provided with a heat drum, provided that exposure and heat development were conducted in the room maintained at 23° C. and 50% RH.

## Evaluation of photographic performance

Images obtained after heat development were evaluated using a densitometer, with respect to a minimum density, Dmin and sensitivity (which is represented as reciprocal of exposure necessary to give a density of 0.1 plus Dmin). The less Dmin, the better. Sensitivity was represented as a relative value, based on the sensitivity of Sample 4 being 100.

## Evaluation of image lasting quality

Samples which were processed in the same manner as in the evaluation of photographic performance were in the dark room maintained at 55° C. and 55% RH over a period of 7 days and visually evaluated with respect to image tone, based on the following criteria:

- 5: No problem in tone,
- 4: Level of no problem in practical use,
- 3: Slightly yellowish but acceptable level,

20 2: Disagreeable tone and unacceptable in practical use,  
1: Marked change in color and unacceptable tone  
Results are shown in Table 2.

25

TABLE 2

| Sample | Emul-sion | Silver salt dis-persion | Dmin | Sensi-tivity | Image lasting quality |       | Remark |
|--------|-----------|-------------------------|------|--------------|-----------------------|-------|--------|
|        |           |                         |      |              | 5                     | 1     |        |
| 1      | E1        | C1                      | 0.18 | 210          | 5                     | Inv.  |        |
| 2      | E2        | C2                      | 0.20 | 205          | 5                     | Inv.  |        |
| 3      | E3        | C3                      | 0.21 | 203          | 5                     | Inv.  |        |
| 4      | E4        | C4                      | 0.23 | 200          | 5                     | Inv.  |        |
| 5      | E5        | C5                      | 0.30 | 180          | 5                     | Inv.  |        |
| 6      | E6        | C6                      | 0.41 | 100          | 1                     | Comp. |        |

30 As apparent from Table 2, inventive samples exhibited superior results in photographic performance and image storage stability.

35 40 What is claimed is:

1. A method for preparing an organic silver salt dispersion comprising the steps of:

- (a) dissolving an organic acid in water at a temperature of 60 to 90° C.,
- (b) adding thereto an alkali to form an aqueous solution or suspension containing an alkali salt of the organic acid,
- (c) cooling the aqueous solution or suspension to a temperature of 0 to 55° C., and then
- (d) adding silver nitrate to the cooled aqueous solution or suspension to form an organic silver salt dispersion, wherein in step (c), the aqueous solution or suspension is cooled at a mean cooling rate of not less than 0.5° C./min.

45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 87

**25**

5. The method of claim 3, wherein said silver halide comprises silver chloride, silver chlorobromide, silver iodochlorobromide, silver bromide, silver iodobromide or silver iodide.

6. The method of claim 3, wherein said silver halide is added in an amount of 0.75 to 30% by weight of the organic silver salt, based on silver.

**26**

7. A thermally processable photosensitive material comprising a support having thereon an organic silver salt, a photosensitive silver halide, a reducing agent and a binder, wherein said organic silver salt is the organic silver salt dispersion prepared by the method as claimed in claim 1.

\* \* \* \* \*